



US008052507B2

(12) **United States Patent**  
**Huang et al.**

(10) **Patent No.:** **US 8,052,507 B2**  
(45) **Date of Patent:** **Nov. 8, 2011**

(54) **DAMPING POLYURETHANE CMP PADS  
WITH MICROFILLERS**

(75) Inventors: **David Picheng Huang**, Westfield, IN (US); **Ming Zhou**, Boxborough, MA (US); **Timothy Dale Moser**, Brownsburg, IN (US)

(73) Assignee: **Praxair Technology, Inc.**, Danbury, CT (US)

(\*) Notice: Subject to any disclaimer, the term of this patent is extended or adjusted under 35 U.S.C. 154(b) by 711 days.

(21) Appl. No.: **11/943,213**

(22) Filed: **Nov. 20, 2007**

(65) **Prior Publication Data**

US 2009/0137120 A1 May 28, 2009

(51) **Int. Cl.**  
**B24D 11/00** (2006.01)

(52) **U.S. Cl.** ..... **451/526**; 156/78; 51/295; 51/296

(58) **Field of Classification Search** ..... **451/526**; 51/296; 264/51

See application file for complete search history.

(56) **References Cited**

U.S. PATENT DOCUMENTS

|              |        |                     |
|--------------|--------|---------------------|
| 3,817,882 A  | 6/1974 | Hostettler et al.   |
| 6,454,634 B1 | 9/2002 | James et al.        |
| 6,514,301 B1 | 2/2003 | Lombardo            |
| 6,582,283 B2 | 6/2003 | James et al.        |
| 6,627,671 B1 | 9/2003 | Kihara et al.       |
| 6,705,934 B1 | 3/2004 | Shiro et al.        |
| 6,777,455 B2 | 8/2004 | Seyanagi et al.     |
| 6,860,802 B1 | 3/2005 | Vishwanathan et al. |
| 6,899,611 B2 | 5/2005 | Reinhardt et al.    |
| 6,918,821 B2 | 7/2005 | Balijepalli et al.  |

|                   |         |                             |
|-------------------|---------|-----------------------------|
| 6,984,163 B2      | 1/2006  | Roberts                     |
| 7,074,115 B2      | 7/2006  | James et al.                |
| 7,097,549 B2      | 8/2006  | Allison et al.              |
| 7,097,550 B2      | 8/2006  | Kawahara et al.             |
| 7,098,255 B2      | 8/2006  | Seyanagi et al.             |
| 7,169,030 B1      | 1/2007  | Kulp                        |
| 7,192,340 B2      | 3/2007  | Ono et al.                  |
| 7,217,179 B2      | 5/2007  | Sakurai et al.              |
| 2004/0157985 A1   | 8/2004  | Masui et al.                |
| 2004/0224622 A1 * | 11/2004 | Sakurai et al. .... 451/526 |
| 2005/0171225 A1   | 8/2005  | Kulp                        |
| 2006/0046064 A1   | 3/2006  | Halberg et al.              |
| 2006/0084365 A1   | 4/2006  | Sakurai et al.              |
| 2006/0226567 A1   | 10/2006 | James et al.                |
| 2006/0254706 A1 * | 11/2006 | Swisher et al. .... 156/253 |
| 2006/0276109 A1   | 12/2006 | Roy et al.                  |
| 2009/0093201 A1   | 4/2009  | Kazuno et al.               |

FOREIGN PATENT DOCUMENTS

WO WO2009/029322 A1 3/2009

\* cited by examiner

*Primary Examiner* — Roberts Culbert

(74) *Attorney, Agent, or Firm* — Nilay S. Dalal

(57) **ABSTRACT**

A system for preparing a microcellular polyurethane material, includes a froth, prepared, for instance, by inert gas frothing a urethane prepolymer, preferably an aliphatic isocyanate polyether prepolymer, in the presence of a surfactant; a filler soluble in a CMP slurry; and a curative, preferably including an aromatic diamine and a triol. To produce the microcellular material, the froth can be combined with the filler, e.g., PVP, followed by curing the resulting mixture. The microcellular material has a low rebound and can dissipate irregular energy and stabilize polishing to yield improved uniformity and less dishing. CMP pads using the microcellular material have pores created by inert gas frothing throughout the pad polymer body and additional surface pores created by dissolution of fillers during polishing, providing flexibility in surface softness and pad stiffness.

**18 Claims, No Drawings**

## 1

DAMPING POLYURETHANE CMP PADS  
WITH MICROFILLERS

## BACKGROUND OF THE INVENTION

Chemical mechanical planarization, also known as chemical mechanical polishing or CMP, is a technique used to planarize the top surface of an in-process semiconductor wafer or other substrates in preparation of subsequent steps or for selectively removing material according to its position. The technique employs a slurry that can have corrosive and abrasive properties in conjunction with a polishing pad.

While many existing CMP pads are non-porous, porous polishing pads generally provide improved slurry transport and localized slurry contact.

One technique for making high density foam polishing pads includes agitating a liquid polymer resin at a controlled temperature and pressure, using a surfactant, to produce a stable froth. The resin froth can be metered under pressure to a mix head where it is typically combined with a desired amount of curative before being injected or poured into a mold.

Other techniques for introducing porosity into pad materials include incorporating beads or hollow polymeric microspheres into the material. In some instances, a polymeric matrix used to manufacture the pad has been combined with polymeric microelements that soften or dissolve upon contact with a polishing slurry.

Many existing CMP pads have pore size limitations imposed by the technique used to create the microstructure. Gas frothing, for instance, can produce wider pore size distributions, larger than 30 microns ( $\mu\text{m}$ ), whereas microspheres-filled pads often have pore sizes greater than 20-30  $\mu\text{m}$ , depending on the size of the microspheres.

Generally, CMP is a dynamic process involving cyclic motion of both the polishing pad and the workpiece. During the polishing cycle, energy is transmitted to the pad. A portion of this energy is dissipated inside the pad as heat, and the remaining portion is stored in the pad and subsequently released as elastic energy during the polishing cycle. The latter is believed to contribute to the phenomenon of dishing of metal features and oxide erosion.

One attempt to describe damping effects quantitatively has used a parameter named Energy Loss Factor (KEL). KEL is defined as the energy per unit volume lost in each deformation cycle. Generally, the higher the value of KEL for a pad, the lower the elastic rebound and the lower the observed dishing.

To increase the KEL value, the pad can be made softer. However, this approach tends to also reduce the stiffness of the pad. The reduced stiffness results in decreased planarization efficiency and increases dishing due to conformation of the pad around the device corner.

Another approach for increasing the KEL value of the pad is to alter its physical composition in such a way that KEL is increased without reducing stiffness. This can be achieved by altering the composition of the hard segments (or phases) and the soft segments (or phases) in the pad and/or the ratio of the hard to soft segments (or phases) in the pad.

## SUMMARY OF THE INVENTION

To address advances in electronic components, increasingly complex demands are being placed on CMP processing and equipment utilized to planarize semiconductor, optical, magnetic or other types of substrates. A need continues to exist for long lasting CMP pads that can provide improved slurry transport and removal rates and can meet requirements

## 2

for within wafer (WIW) and within die (WID) uniformities. Also needed are pads that are less likely to cause scratching, dishing and/or erosion, as well as pads that require less conditioning.

5 It has been found that CMP pads with low rebound tend to absorb relatively high amounts of energy during cyclic deformation, causing less dishing during polishing and yielding better WID uniformity. Stiffness is an important consideration for WID uniformity and prolonged pad life, while 10 decreased glazing during polishing reduces the need for pad conditioning.

The invention relates to producing CMP pad materials that have special properties, in particular a highly damping performance and/or improved pore structure at the working surface. 15 These and other properties are obtained by altering the formulation and process for producing the pad. Choices in ingredients and specific combinations of materials, together with processes such as gas frothing have been found to affect the morphology of the polymeric material, resulting in a final 20 product that has properties that are particularly advantageous in fabricating CMP pads.

In one aspect, the invention is directed to a system and method for producing a microcellular polyurethane material.

25 The system includes a urethane prepolymer, a curative and a filler. When combined under polymerization conditions the urethane prepolymer, the curative and the filler form a solid product having a Bashore rebound that is less than 38%.

The method includes frothing a urethane prepolymer to 30 form a froth, incorporating a filler in the froth and curing the froth in the presence of a curative, thereby producing the microcellular polyurethane material, wherein a solid product formed by polymerizing the urethane prepolymer and filler in the presence of the curative has a Bashore rebound that is less than 38%.

35 It was discovered that systems that are combinations of polyether urethane prepolymers that contain aliphatic isocyanates, such as H12MDI or HDI, and curatives that include aromatic diamines tend to form highly damping polyurethane materials. It was further discovered that adding triol, e.g., to 40 the aromatic diamine, tended to decrease the Bashore rebound of a solid material formed by polymerizing the prepolymer and curative. In addition to the pore structure generated by gas frothing, fillers that dissolve in a CMP slurry can add a second pore structure at the polishing or working surface of the pad.

45 In a preferred implementation of the invention, a system for producing a CMP pad comprises a froth that includes an inert gas, an aliphatic isocyanate polyether prepolymer, a polysiloxane-polyalkyleneoxide surfactant, a slurry-soluble filler and a curative that preferably includes an aromatic diamine. The particle size of the filler can be selected to impart a dual porosity at the working surface of the pad. In specific embodiments, the system also includes a triol, for instance as part of the curative. Triol levels can be optimized for higher damping 50 performance.

55 In another preferred implementation of the invention, a method for producing a CMP pad includes frothing an aliphatic isocyanate polyether prepolymer with an inert gas, in the presence of a polysiloxane-polyalkyleneoxide surfactant, to form a froth; adding a slurry-soluble filler to the froth; and curing the filler-containing froth in the presence of a curative, e.g., an aromatic diamine and a triol.

60 The invention addresses demands placed on CMP pads used in the manufacture of traditional and advanced electronic, optical or magnetic components and has many advantages. The highly damping polymeric material of the invention has high energy dissipation and can absorb irregular

bouncing and oscillating energy at the polishing interface to yield better uniformity. CMP pads manufactured from this material provide good WIW and WID uniformities, smooth polishing performance, low dishing and/or erosion. The pads generally have a high degree of stable hardness or stiffness, providing good planarization performance and long pad life. During operation, CMP pads fabricated from the highly damping microcellular materials described herein can absorb irregular bouncing and oscillating energy at the polishing interface, giving smooth polishing performance and low dishing/erosion on wafer surface.

The slurry soluble filler employed according to the invention can generate a second porosity at the CMP polishing interface resulting in decreased glazing and requiring less conditioning. Filler-induced porosity at the pad surface can retain additional slurry while fillers inside the pad body can change the hardness of pad resulting in gradient of porosity and hardness from top down of the polymer pad, thereby yielding improved WID uniformity during polishing. In preferred examples, the dual porosity distributions at the pad surface provides a flexibility in regulating surface pore size for retaining slurry. The dual porosity combination created by gas frothing and soluble fillers can be custom designed or optimized for specific polishing applications depending on the needs for removal rate and surface finish. The dual surface porosity described herein can require less microcellular porosity within the bulk material, making the pad stiffer (harder) and giving excellent polishing planarity.

By providing a wide range of particle sizes, fillers that dissolve in the CMP slurry can produce desired void sizes at the working interface, thus overcoming pore size limitations in existing CMP pads.

Testing and comparing material properties can be simplified by using solid products, formed by combining a urethane prepolymer with a curative under polymerization conditions, rather than microcellular samples which require additional process steps, e.g., frothing, and/or ingredients, e.g., surfactants.

Advantageously, the material can be prepared using precursors that are commercially available thus simplifying and facilitating the overall fabrication process. Aspects of gas frothing and casting can be carried out using standard techniques and/or equipment. In some systems, frothing time can be decreased without sacrificing foaming characteristics and quality.

#### DETAILED DESCRIPTION OF THE PREFERRED EMBODIMENTS

The above and other features of the invention including various details of construction and combinations of parts, and other advantages, will now be more particularly described with reference to the accompanying drawings and pointed out in the claims. It will be understood that the particular method and device embodying the invention are shown by way of illustration and not as a limitation of the invention. The principles and features of this invention may be employed in various and numerous embodiments without departing from the scope of the invention.

In one aspect, the invention relates to a damping polymeric material that is particularly well suited in the manufacture of CMP pads. As used herein, the term "damping" refers to the ability of a material to absorb mechanical energy. Preferably damping is measured by the Bashore rebound method, a simple technique for testing the rebound of a material. The Bashore rebound test is known in the art and is described, for instance, in the American Society for Testing and Materials

(ASTM) Standard D-2632. Other methods for measuring rebound also can be used, as known in the art.

The polymeric material is a polyurethane, i.e., a polymer containing repeating urethane units. The polyurethane is produced from a system that includes at least one urethane prepolymer and a curative. The system can include other ingredients, e.g., surfactants, fillers, catalysts, processing aids, additives, antioxidants, stabilizers, lubricants and so forth.

Urethane prepolymers are products formed by reacting 10 polyols, e.g., polyether and/or polyester polyols, and difunctional or polyfunctional isocyanates. As used herein, the term "polyol" includes diols, polyols, polyol-diols, copolymers and mixtures thereof.

Polyether polyols can be made through alkylene oxide 15 polymerization and tend to be high molecular weight polymers, offering a wide range of viscosity and other properties. Common examples of ether-based polyols include polytetramethylene ether glycol (PTMEG), polypropylene ether glycol (PPG), and so forth.

Examples of polyester polyols include polyadipate diols, polycaprolactone, and others. The polyadipate diols can be made by the condensation reaction of adipic acid and aliphatic diols such as ethylene glycol, propylene glycol, 1,4-butanediol, neopentyl glycol, 1,6-hexanediol, diethylene glycol and mixtures thereof.

Polyol mixtures also can be utilized. For instance, polyols such as those described above can be mixed with low molecular weight polyols, e.g., ethylene glycol, 1,2-propylene glycol, 1,3-propylene glycol, 1,2-butanediol, 1,3-butanediol, 30 2-methyl-1,3-propanediol, 1,4-butanediol, neopentyl glycol, 1,5-pentanediol, 3-methyl-1,5-pentanediol, 1,6-hexanediol, diethylene glycol, dipropylene glycol and mixtures thereof.

The most common isocyanates utilized in preparing urethane prepolymers are methylene diphenyl diisocyanate (MDI) and toluene diisocyanate (TDI), both aromatic. Other aromatic isocyanates include para-phenylene diisocyanate (PPDI), as well as mixtures of aromatic isocyanates.

In specific aspects of the invention, the urethane prepolymers employed include aliphatic isocyanates such as, for 40 instance, hydrogenated MDI (H12MDI), hexamethylene diisocyanate (HDI), isophorone diisocyanate (IPDI), other aliphatic isocyanates and combinations thereof.

Urethane prepolymers also can include mixtures of aliphatic and aromatic isocyanates.

Urethane prepolymers often are characterized by the weight percent (wt %) of unreacted isocyanate groups (NCO) present in the prepolymer. Wt % NCO can be used to determining mixing ratios of components for producing polyurethane materials.

Urethane prepolymers can be formed using synthetic techniques known in the art. In many cases, suitable urethane prepolymers also are commercially available.

Examples of commercially available polyether urethane prepolymers include some Adiprene® polyether prepolymers, from Chemtura Corporation, Middletown, Conn., some Airthane® prepolymers, from Air Products and Chemicals, Inc. Allentown, Pa., and others. In many cases, these prepolymers contain low levels of free monomer, e.g., TDI monomer, and are referred to as "low free" or "LF".

Specific examples of polyether urethane prepolymers include, for instance, those designated as (Adiprene®) LF 750D (a TDI-PTMEG prepolymer, LF, having a NCO of 8.79 wt %), L 325 (TDI/H12MDI-PTMEG prepolymer, having a NCO of 9.11 wt %), LFG 740D (TDI-PPG prepolymer, LF, having a NCO of 8.75 wt %), LW 570 (H12MDI-polyether prepolymer, having a NCO of 7.74 wt %), LFH 120 (HDI-polyether prepolymer, LF, having a NCO of 12.11 wt %) and

Airthane® PHP-80D (TDI-PTMEG prepolymer, LF, having a NCO of 11.1 wt %). Other specific examples of urethane prepolymers that are commercially available include Andur® (Anderson Development Company), Baytec® (Bayer Material Science) and so forth.

Examples of polyester urethane prepolymers include, for instance, a TDI polyester urethane prepolymer designated as Vibrathane® 8570, having a NCO of 6.97 wt %, from Chemtura Corporation, Middletown, Conn. Other suitable polyester urethane prepolymers include but are not limited to Verathane® D-6 or D-7 from Air Products and Chemicals.

The curative is a compound or mixture of compounds used to cure or harden the urethane prepolymer. The curative reacts with isocyanate groups, linking together chains of prepolymer to form a polyurethane.

Common curatives typically used in producing polyurethane include 4,4'-methylene-bis(2-chloroaniline), abbreviated as MBCA and often referred to by the tradename of MOCA®; 4,4'-methylene-bis-(3-chloro-2,6-diethylaniline), abbreviated as MCDEA; dimethylthiotoluenediamine, trimethyleneglycol di-p-aminobenzoate; polytetramethyleneoxide di-p-aminobenzoate; polytetramethyleneoxide mono-p-aminobenzoate; polypropyleneoxide di-p-aminobenzoate; polypropyleneoxide mono-p-aminobenzoate; 1,2-bis(2-aminophenylthio)ethane; 4,4'-methylene-bis-aniline; diethyltoluenediamine; 5-tert-butyl-2,4- and 3-tert-butyl-2,6-toluenediamine; 5-tert-amyl-2,4- and 3-tert-amyl-2,6-toluenediamine and chlorotoluenediamine and others.

In specific aspects of the invention, the curative employed includes an aromatic amine, in particular an aromatic diamine, e.g., bis-(alkylthio) aromatic diamines. Commercial examples of suitable aromatic diamines include Ethacure® 300 (from the Albermarle Corporation, Richmond, Va.), which is a mixture containing 3,5-bis(methylthio)-2,6-toluenediamine and 3,5-bis(methylthio)-2,4-toluenediamine; and Ethacure® 100 (also from Albermarle Corporation) which is a mixture containing 3,5-diethyltoluene-2,4-diamine and 3,5-diethyltoluene-2,6-diamine.

In addition to the aromatic diamine component, preferred curatives include one or more other ingredients. For instance, to modify the urethane domain network or polymer structure, polymer cross-linking density is increased by introducing tri-functional agents for damping performance. Preferred examples of trifunctional agents include triols, for instance aliphatic triols such as trimethanolpropane (TMP), alkoxylated aliphatic triols, e.g. ethoxylated TMP, such as TP30, available from Perstorp Corporation, polypropylene ether triol having, for instance, a molecular weight of 100-900 and aliphatic amino triols such as Vibracure® A931, available from Chemtura, triethanol amine (TEA), and others. Mixtures of triols also can be employed.

Triol levels can be optimized for damping performance. Relative to the entire weight of the curative, triols or modified triols, e.g., alkoxylated triols, typically are used in an amount within the range of from 0.2 to 15 weight %. Other ratios can be employed.

In specific examples, the preferred curative for use with aliphatic (HDI or H12MDI) polyether urethane prepolymers is a mixture of Ethacure® 300 in combination with 5-10% wt triol, and in particular the combination of Ethacure 300 with 5% TMP.

Relative amounts of urethane prepolymer and curative can be determined, for instance, by taking into account the % NCO of a given urethane prepolymer. The curative can be added to give a combination of amine and hydroxyl groups at about, e.g., 95%, of the available isocyanate groups in the

prepolymer on an equivalent basis. In most instances, curative is added at 90-105% the theoretical amount.

In other embodiments, triol can be added individually or with ingredients other than the curative.

5 The Bashore rebound preferably is measured using a solid product obtained by combining a urethane prepolymer and a curative under polymerization conditions, e.g., suitable temperatures and time periods to cure or harden the combination into a solid product. Generally, the solid product is formed 10 without subjecting the prepolymer to a process intended to introduce microscopic sized voids into the material, for example in the absence of frothing, further discussed below.

Preferred prepolymer-curable combinations polymerize to form a solid product that has a rebound less than about 15 38%, as measured by the Bashore rebound test. Highly damping solid products, e.g., having a rebound lower than 35%, were obtained from systems that include H12MDI or HDI polyether prepolymers and a curative that is a mixture of Ethacure® 300 and 5 weight % TMP.

20 The solid product can be used to screen candidate systems with respect to other properties such as hardness. In preferred examples, the solid product has a hardness in the range of from about 30 D to about 85 D, e.g., from 55 D to 80 D. The Shore D scale, utilizing Durometer testing, is a well known 25 approach for defining hardness of polymeric materials and generally is applied to plastics harder than those measured on the Shore A scale. The Shore D hardness was measured according to ASTM D 2240.

Other properties that can be studied and compared using a 30 solid product formed by combining a urethane prepolymer and a curative under polymerization conditions include processability, i.e., the ability to form froth and mixing, chemical stability of the product vis-à-vis slurries employed in CMP processing, viscosity of the system, release of free monomer, 35 e.g., TDI, during processing, pot life, color, and so forth.

For manufacturing CMP pads, the polyurethane material is microcellular, containing microscopically sized voids which typically are formed by processes targeted at incorporating such voids into the structure of the material. During CMP 40 planarization, the voids or micropores retain slurry for polishing the surface of the workpiece.

In specific aspects of the invention, at least a portion of the void volume is formed by frothing with a gas such as nitrogen, dry air, rare gases, e.g., helium, argon, xenon, as well as other 45 gases or gas mixtures. Gases that do not cause chemical reactions such as oxidation reactions in the foam are preferred and are referred to herein as "non-reactive" or "inert" gases. Particularly preferred is nitrogen.

Frothing is described, for instance, in U.S. Pat. No. 6,514, 50 301B, issued to Brian Lombardo on Feb. 4, 2003, the teachings of which are incorporated herein by reference in their entirety. Preferably, frothing produces microstructures with adjustable pore size and distribution. In one example, the microcellular polyurethane material has pores greater than 55 about 30  $\mu\text{m}$ .

Frothing the prepolymer can be conducted in the presence of one or more surfactant(s), e.g., non-ionic or ionic surfactant(s). Including a surfactant can be particularly beneficial in systems having low viscosity.

60 A stable froth (foam) is preferred in creating microstructure in polyurethane materials and is believed to result, at least in part, from the adsorption and partition of hydrophobic hydrocarbon chains of surfactant at the air/polymer interface causing changes in surface tension and reaction of its functional group with the polymer.

It is desirable to select a surfactant which, when used with a specific urethane prepolymer, easily produces froth, prefer-

ably using simple processing and equipment. Froths that are stable and maintain their integrity when subjected to varying processing conditions, e.g., shear, temperature or pressure variations, typically employed during processing also are preferred. It was also found that surfactant selection could affect not only frothing intensity or froth stability but also pore size, an important parameter for polymeric materials used to manufacture CMP pads.

Examples of suitable surfactants include silicone surfactants such as, for instance, copolymers containing at least one block comprising polydimethylsiloxane and at least one other block comprising polyether, polyester, polyamide, or polycarbonate segments.

In specific embodiments the surfactant is a polysiloxane-polyalkyleneoxide (or polysiloxane-polyalkylene oxide) surfactant. Polysiloxane-polyalkyleneoxide surfactants also are known in the art as a silicone copolymers and can include polymeric, oligomeric, copolymeric and other multiple monomeric siloxane materials.

Polysiloxane-polyalkyleneoxide surfactants can be copolymers that comprise a polysiloxane backbone comprised of siloxane units, and polyalkyleneoxide sidechains. The polysiloxane backbone can be either straight chain, branched chain or cyclic in structure. The polyalkyleneoxide sidechain of copolymers may include polyethyleneoxide, polypropyleneoxide, polybutyleneoxide macromonomers and so forth, or mixtures thereof. Optionally, the sidechains may also include polyethylene, polypropylene, polybutylene monomers. The polyalkyleneoxide monomer can be present in an amount greater than about 10%, preferably greater than about 20%, and more preferably greater than about 30% by weight of the copolymer.

Polyethyleneoxide sidechain macromonomers are preferred. Also, preferred are polypropyleneoxide sidechains, and sidechains comprising polyethyleneoxide and polypropylene oxide at a mole ratio of from about 1:2 to about 2:1.

Particularly useful are copolymers having a molecular weight ranging from about 2,000 to about 100,000 g/g-mole, preferably from about 10,000 to about 80,000 g/g-mole, more preferably from about 15,000 to about 75,000, even more preferably from about 20,000 to about 50,000, and most preferably from about 25,000 to about 40,000.

The polysiloxane-polyalkyleneoxide copolymers of the present invention can have a surface tension of less than about 40 mN/m, preferably less than about 30 mN/m, and more preferably less than about 25 mN/m. The surface tension is measured by the Wilhelmy plate test method according to ASTM D1331-89 using a 0.1% by weight solution at 25° C.

The copolymers can have a Ross Miles foam height of less than about 60 millimeters (mm), preferably less than about 40 mm, more preferably less than about 20 mm, and most preferably less than about 10 mm. The Ross Miles foam height test is performed according to ASTM C1173-53 using 1% by weight solutions and taking 5 minute readings. Additionally, the copolymers can have a hydrophile-lipophile balance (HLB) greater than or equal to about 4, preferably greater than or equal to about 6, and more preferably greater than or equal to about 8.

Examples of commercially available surfactants that can be used are some available from GE Silicones under the designation of Niax®, for instance L-7500, L-5614, L-1580; from Air Products and Chemicals, e.g., under the designation of DC-193, DC-5604 and DC-5164; and from Dow Corning Corporation, Midland, Mich., e.g., under the designation DC-309, 5098EU and Q2-5211 (methyl(propylhydroxide, ethoxylated) bis(trimethylsiloxy)silane).

The surfactant preferably is selected based on parameters such as foaming intensity, stability or cell size obtained during frothing. For many urethane prepolymers that include aromatic isocyanates, a suitable surfactant is Niax® L-1800 (a polydimethylsiloxane polyoxyalkylene block copolymer surfactant) available from GE Silicones, now Momentive Performance Materials. Preferred surfactants for frothing aliphatic isocyanate polyether prepolymers, e.g., H12MDI-polyether or HDI-polyether, include DC-193 and Q2-5211.

Amounts of surfactant can be determined experimentally, for instance by evaluating frothing characteristics and/or properties of the end product. Typically, surfactant levels are within the range of from about 0.3 to about 5% by weight with respect to the total weight of prepolymer and surfactant. Surfactant amounts also can be expressed as parts per hundred parts of resin (PHR). In many cases, a suitable surfactant amount was around 1.5 PHR. Other amounts can be selected.

The system also includes at least one filler that is soluble in the slurry employed during CMP polishing. More than one type of slurry-soluble fillers can be employed.

Generally, the slurry provides mechanical as well as chemical action by combining abrasives and compounds that can chemically affect the substrate being planarized. Many CMP slurries are aqueous-based formulations developed for specific applications and can include pH adjusters, chelating agents, lubricants, surface modifiers, corrosion inhibitors and so forth. Examples of abrasives that can be utilized are colloidal or precipitated silicas, fumed metal oxides, e.g., silica or alumina, polymeric spheres, nanoparticles, e.g., ceria, and many others.

Slurries designed to remove insulating materials, for instance, often contain water, an abrasive and an alkali formulation for hydrolyzing the insulating material. Copper slurries on the other hand, can include water, an abrasive, an oxidizing agent and a complexing agent. Abrasive-free slurries also have been developed and are becoming increasingly available.

Upon contact with the slurry, dissolution of the filler increases the porosity at the working surface of the pad. The voids generated by filler particles that have dissolved in the slurry can have characteristics, e.g., pore size, pore distribution, pore forming speed, that are different from the voids introduced by gas frothing, resulting in a dual pore structure at the working surface of the pad.

Fillers that are soluble in the CMP slurry, can be provided in a particle size suitable for the application. To generate a dual porosity at the working surface, the particle size of the filler(s) preferably is different from the cell size introduced in the material by gas frothing. Multiple porosities can be imparted to the working surface by using filler(s) in two or more particle sizes that are different from the cell size formed throughout the material by frothing.

Fillers having a particle size that is the same or essentially the same as the pore size generated by frothing also can be employed.

In many cases, the filler has a particle size, e.g., an average particle size in the range of from about 1  $\mu$ m to about 100  $\mu$ m, preferably from about 5  $\mu$ m to about 80  $\mu$ m. In specific examples, the filler has an average particle size within the range of from about 20  $\mu$ m to about 50  $\mu$ m.

For aqueous CMP slurries, preferred fillers are water-soluble. Examples include fillers made of organic water-soluble materials, such as saccharides, polysaccharides, e.g., starch, dextrin and cyclodextrin, lactose, mannitol, etc., celluloses, e.g., hydroxypropyl cellulose, methyl cellulose, etc., proteins, polyvinyl alcohol, polyacrylic acid and salts thereof, polyethylene oxide, water-soluble photosensitive resins, sul-

fonated polyisoprene and sulfonated polyisoprene copolymers. Inorganic water-soluble fillers such as, for instance, potassium acetate, potassium nitrate, potassium carbonate, potassium hydrogencarbonate, potassium chloride, potassium bromide, potassium phosphate, magnesium nitrate and others also can be used.

In specific embodiments, the slurry-soluble filler does not dissolve in ingredients employed to form the microcellular material. In other specific embodiments, the filler affects chemical reactions, e.g., cross-linking, taking place during the preparation of the microcellular material. For instance, the filler can react with the pre-polymer, the curative or both during frothing and/or curing step(s).

A preferred filler is polyvinylpyrrolidone or PVP. PVP is a vinyl polymer that can be prepared by free radical polymerization of the monomer vinylpyrrolidone. Its chemical structure is represented by the formula:



PVP is soluble in water and in solvents such as ethanol and others and is used in pharmaceutical, cosmetic and personal care formulations as well as in other applications.

Commercially, it is available in solution as well as in powder form. As known in the art, particle sizes of granular materials can be controlled, e.g., by sieving. Suitable average particle sizes are in the range of from about 1  $\mu\text{m}$  to about 100  $\mu\text{m}$ , preferably from about 5  $\mu\text{m}$  to about 80  $\mu\text{m}$ . In specific examples, the average PVP particle size is within the range of from about 20  $\mu\text{m}$  to about 50  $\mu\text{m}$ .

PVP can be obtained, for example, from BASF Corporation, Florham Park, N.J., under the designation of Luvitec® K-15, K-30, K-60 and K-90. These products have different viscosity grades and average molecular weights of about 10,000, 40,000, 60,000 and 360,000, respectively.

Filler amounts can be selected to produce a desired porosity at the interface of the microcellular material and the work-piece. While filler concentrations that are too low can result in insufficient porosity, concentrations that are too high can lead to aggregation and loss of pore uniformity. Based on the total weight of the pad, the slurry soluble filler can be present in an amount in the range of from about 0.2 to about 40 wt %, preferably from about 1 to about 20 wt %. In one preparative example, based on the total weight of prepolymer, surfactant, filler and curative, the filler is present in an amount within the range of from about 1 to about 20 wt %.

The filler can be combined with any of the ingredients and at any stage of forming the microcellular material. Preferably, at least a portion of the filler is combined with a froth produced, e.g., by gas frothing of the urethane prepolymer in the presence of a surfactant.

A particularly preferred system includes an aliphatic isocyanate polyether prepolymer; a polysiloxane-polyalkylene oxide surfactant; a filler soluble in a CMP slurry; a curative that includes an aromatic diamine; and, optionally, a triol.

The system used for forming the polymeric material optionally can include other ingredients, such as catalysts, additional fillers, processing aids, e.g., mold release agents, additives, colorants, dyes, antioxidants, stabilizers, lubricants and so forth.

Catalysts, for instance, are compounds that are added, typically in small amounts, to accelerate a chemical reaction without being consumed in the process. Suitable catalysts that can be used to produce polyurethane from prepolymers include amines and in particular tertiary amines, organic acids, organometallic compounds such as dibutyltin dilaurate (DBTDL), stannous octoate and others.

Additional fillers can be added to further affect polishing properties of a CMP pad, e.g., material removal rates, to promote porosity or for other reasons. Specific examples of suitable fillers include but are not limited to particulate materials, e.g., fibers, hollow polymeric microspheres, functional fillers, nanoparticles and so forth.

In another aspect, the invention relates to preparing a microcellular polyurethane material. In a preferred process, a urethane prepolymer is combined with a surfactant and frothed to produce a froth which will be cured in the presence of a curative. A filler that is soluble in a CMP slurry, e.g., PVP, is included. The slurry-soluble filler can be added at any stage of the preparation process.

In specific examples, the filler is added at the frothing stage, e.g., before, during and preferably after formation of the froth. Preferred froth-filler combinations and amounts produce uniform microcellular structure, with reduced cell of filler clustering. Froth-filler mixing can be conducted using paddles, stirrers, propellers, agitators, vortex mixers or other suitable mixing devices.

One or more optional ingredient(s) e.g., catalysts, fillers, processing aids, additives, dyes, antioxidants, stabilizers, lubricants and so forth can be added to or can be present in the prepolymer, curative or surfactant. One or more such ingredients also can be added during frothing or to the resulting foam.

Frothing can be conducted with nitrogen or another suitable gas, using equipment such as commercial casters with pressurized or non-pressurized tanks and distribution system or other mixing systems.

The structure imparted by frothing includes gas bubbles, also referred to herein as voids or pores, that are introduced into the material being frothed, and these can be characterized by a mean pore size, pore count and/or pore surface area percentage. Uniform bubbles are preferred as are microscopic mean pore sizes.

In many instances, typical frothing temperatures can be within the range of from about 50 to about 230° F., e.g., 130 to about 185° F.; frothing time can be within the range of from about 12 to about 240 minutes; gas, e.g., nitrogen, flow can be within the range of from about 1 to about 20 standard cubic feet per hour; mixing speed can be within the range of from about 500 to about 5000 rotations per minute (RPM).

The pot can be maintained at ambient conditions or under pressure, e.g., up to about 10 atmospheres.

The froth is cast and cured in the presence of the curative to produce the polyurethane material.

Casting can be conducted by pouring the foam into a mold, for instance a mold suitable for producing a desired CMP pad. Mold dimensions and shapes useful in manufacturing CMP pads are known in the art.

Curing or hardening the froth to produce a microcellular polyurethane material can be carried out in an oven, e.g., a box oven, convey oven or another suitable oven, at a suitable curing temperature and for a suitable period of time. Systems such as described above can be cured at a temperature in the range of from about 50 to about 250° F., e.g., 235° F., for a period of time of about 30 minutes. The curing process and its end point can be determined by evaluating the viscosity and hardness of the system.

## 11

Curing can be conducted in air or under special atmospheres, e.g., nitrogen, or another suitable gas or gas mixture.

After it is determined that curing is completed, for instance at the point when the system in the mold can no longer be poured, the hardened microcellular product is released from the mold and can be post-cured in an oven at a suitable temperature and for a suitable period of time. For instance the hardened product can be post-cured at a temperature within the range of from about 200 to about 250° F. e.g., 235° F. for several hours, e.g., 8-16.

Following post-curing, the microcellular product also can be conditioned at room temperature for a period of several hours to a day or longer.

In one example of the invention, gas, e.g., inert gas is used to form a froth containing gas, aliphatic isocyanate polyether prepolymer and polysiloxane-polyalkylene oxide surfactant. The froth is combined with the filler and the resulting composition is cured in the presence of the curative and optional triol.

The microcellular material described herein preferably has a Bashore rebound within the range of from about 25% to about 50%. In specific examples, the Bashore rebound of the microcellular material is less than 36%.

The material can have a density within the range of from about 0.6 to about 1.0 g/cm<sup>3</sup>, preferably within the range of from about 0.80 to about 0.95.

In some embodiments, the hardness of the microcellular polymeric material is in the range of from about 30 to about 80 D.

Within the body of the material, the porous structure generated by frothing preferably has a cell size, also referred to as "pore" size, that is uniform throughout the material. The mean pore size of this first pore structure can be in the range of from about 2 microns (μm) to about 200 μm. In some specific instances, the mean pore size is greater than about 30 microns (μm), for example within the range of from about 50 to about 100 μm and larger, e.g., up to about 120 μm and higher. Pore area % can range from about 5% to about 60%.

Upon contact with a CMP slurry, additional pore structure can be created at the working surface by dissolution of the slurry-soluble filler. The pore size of this secondary pore structure can be the same or different from the pore size of the first, i.e., frothing induced, pore structure.

In one example, the working surface has (a) cells of about 35 μm created through gas frothing; and (b) cells of about 10 μm formed by dissolving a slurry-soluble filler having a particle size of about 10 μm. Other dual or multiple porosities can be generated at the surface of the pad to meet requirements of specific polishing applications, removal rates and/or defect performance.

Without wishing to be held to a particular mechanism or interpretation, it is believed that frothing with a non-reactive gas, e.g., nitrogen or another inert gas, in the presence of surfactant affects pore distribution and size during foaming. During frothing, the surfactant appears to control pore size and distributions by controlling surface tension at the air/liquid interface. Fillers such as PVP may contribute to properties of the microcellular material, for example by participating in or affecting physical and chemical processes taking place during frothing and/or curing.

CMP pads manufactured using a system and method such as described above can be utilized with slurries designed for polishing copper as well as aluminum-based electronic components, in the planarization or polishing of semiconductors, optical, magnetic or other substrates. During polishing, the slurry-soluble filler dissolves in the slurry, generating voids at the working surface of the pad. Whereas the body of the pad

## 12

includes pores introduced during frothing, the pad working surface has not only porosity generated by frothing but also porosity resulting from dissolution of the slurry-soluble filler. Controlling frothing conditions, choice of surfactant, filler particle size, filler concentration and/or other parameters can combine to design pads having desired rebound and pore structure.

## Exemplification

10 General Prepolymer Casting Procedure  
15 150-200 grams of each prepolymer were weighed into a pre-weighed pint tin can (~500 ml). The tin can was placed on a hot plate and the contents were heated to 70° C., as monitored by a thermometer, while stirring. The tin can was then placed in a vacuum chamber to remove any dissolved gases for about 3-5 minutes. The temperature of the prepolymer was measured again with the thermometer and was maintained at 60° C. If needed, the prepolymer was heated again on the hot plate. The actual weight of the prepolymer in the tin can was measured accurately on a scale by subtracting the weight of the tin can from the total weight.

20 25 Curative was poured into the can of prepolymer on the scale within 30 seconds and a timer was pressed immediately. Unless otherwise indicated, the curative was added at a level to give a combination of amine and hydroxyl groups at about 95% of the available isocyanate groups in the prepolymer on an equivalent basis.

25 30 After the desired amount of the curative had been added, the system was hand-mixed gently, using a spatula (1.5"×6") for about one minute, to minimize air bubble entrapping. The mixture was then poured into button or slab aluminum molds, pre-sprayed with mold release agent, and preheated to 235° F. in a box oven. Seven (7) buttons having a diameter 1" and a height of 0.5" were prepared. Elastomeric sheets prepared were about 1/16" or 1/4 inch thick.

35 40 45 Curing was conducted in a box oven at 235° F. The pot life of the mixture was monitored until the mixture in the tin could not be poured. After 10 minutes, the button mold was taken out from the oven and the top portions of the button samples were cut with a utility knife to test the easiness of the cutting and the brittleness or strength of the material at this green curing stage. Both button and slab molds were de-molded at about 20-30 minutes to check the de-moldability.

45 50 The buttons and sheets were then post-cured for about 16 hours at 235° F. They were conditioned at room temperature for at least 1 day before hardness and rebound tests and for at least 7 days before any other physical testing.

## Prepolymer Frothing with Surfactant Choice

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9

rim by a ruler for frothing volume monitoring. After 45-120 minutes of frothing, the liquid level was measured again for the frothing volume calculation using the known can diameter (typical 30% increase). The frothed prepolymer was manually cast with the chosen curative within 30 minutes and kept in an oven at a temperature of 150° F.

#### Frothed Prepolymer Cast with Curative Choice

About 150 g of the frothed prepolymer at 150° F. was poured into a dry pint tin can (de-rimmed). Stopwatch timing was started and the calculated amount of the curative choice, e.g. ET5 (95% E300+5% TMP), in a 500 ml brown glass bottle kept in 150° F. oven for use was added into the pint can with a disposable plastic pipette in about 40 seconds.

Mixing the mixture in the can with a 1.5 inch-wide metal spatula was immediately started and was continued for one minute, avoiding any air bubble entrapment. The reaction mixture was poured into two molds: 1 inch button mold and  $\frac{1}{16}$  inch slab mold, both pre-wiped with Stoner M800 mold release agent and pre-heated at 235° F. in an oven before casting.

Both filled molds were placed in a box oven at 235° F. The timing was closely monitored and the mixture viscosity in the can was frequently checked with the spatula until it was no longer possible to pour the mixture for the pot life measurement which was typically 6-7 minutes. After 10 minutes, the flat portions of the button samples were cut off with a utility knife to check cutting processability. Both button and slab samples were demolded in about 30 minutes from the mixing point. The demolded samples were placed in 235° F. oven for a 16 hour post curing period. The button samples were used to measure hardness (Shore D), rebound (Bashore), density and porosity. For hardness and rebound measurements, the button samples were conditioned at ambient temperature for 1+ day.

#### Materials

The urethane prepolymers employed in the experiments described below were obtained commercially and included: Adiprene®) LF 750 D (a TDI-PTMEG prepolymer, LF, having a NCO of 8.79 wt %); Airthane® PHP-80D (TDI-PTMEG prepolymer, LF, having a NCO of 11.1 wt %); L 325 (TDI/H12MDI-PTMEG prepolymer, having a NCO of 9.11 wt %); LFG 740D (TDI-PPG prepolymer, LF, having a NCO of 8.75 wt %); LW 570 (H12MDI-polyether prepolymer, having a NCO of 7.74 wt %); and LFH 120 (HDI-polyether prepolymer, LF, having a NCO of 12.11 wt %). The prepolymers are listed in Table A and are identified by their commercial name, chemical composition, supplier, and % NCO.

TABLE A

| Pre-polymer ID | Commercial Name | Isocyanate | Polyol Backbone | Supplier     | % NCO |
|----------------|-----------------|------------|-----------------|--------------|-------|
| A              | LF750D          | TDI, LF    | polyether       | Chemtura     | 8.79  |
| B              | PHP-80D         | TDI, LF    | polyether       | Air Products | 11.1  |
| C              | L325            | TDI/H12MDI | polyether       | Chemtura     | 9.11  |
| D              | LFG740D         | TDI, LF    | PPG             | Chemtura     | 8.75  |
| E              | LW570           | H12MDI     | polyether       | Chemtura     | 7.74  |
| F              | LFH120          | HDI, LF    | polyether       | Chemtura     | 12.11 |
| G              | 8570            | TDI        | polyester       | Chemtura     | 6.97  |

#### Example 1

Several curatives were evaluated for each of the polyurethane prepolymers identified as A through G in Table A. The curative tested included a commercially aromatic diamine identified herein as MOCA; Ethacure® 300 (from Alber-

marle Corporation) identified herein as E300, Ethacure® 100 (from Albermarle Corporation), identified herein as E100; butanediol, abbreviated herein as BDO; and several mixtures of aromatic diamines and triols, abbreviated as EP10, EA10, ET5, ET10, E1T5 and E1T10, and defined as follows:

$$EP10 = E300 + 10\% TP30$$

$$EA10 = E300 + 10\% A931$$

$$ET5 = E300 + 5\% TMP$$

$$ET10 = E300 + 10\% TMP$$

$$E1T5 = E100 + 5\% TMP$$

$$E1T10 = E100 + 10\% TMP$$

where TMP is trimethanolpropane, TP30 is modified TMP and A931 is an aliphatic amino triol. Percentages are weight percentages.

Table 1 lists systems that were studied, each system corresponding to a combination of a specific urethane prepolymer and a specific curative. Table 1 identifies each system by the letter corresponding to the urethane prepolymer (from Table A), followed by a numeral related to the specific curative employed. For instance, system E5 included the aliphatic isocyanate polyether prepolymer LW570 and the curative ET5; system F3 included the aliphatic isocyanate polyether prepolymer LFH120 and the curative ET5; and G2 included the aromatic isocyanate polyester prepolymer 8570 and the curative E300.

The solid product obtained by combining, under polymerization conditions, the specific prepolymer with the specific curative in each system was evaluated with respect to hardness and Bashore rebound. In some cases, other parameters such as processability and CMP slurry immersion also were studied.

The solid product obtained using system C1, where the prepolymer was L325 and the curative was MOCA is a comparative material formed using L325-MOCA. Microsphere fillers are added when the material is fabricated into a polishing pad.

Sample A2 (LF750D and MOCA) had a Bashore rebound of 42% and was used as a benchmark.

TABLE 1

| System ID | Prepolymer | Curative | % Theory (%) |    | Bashore Rebound (%) |
|-----------|------------|----------|--------------|----|---------------------|
|           |            |          | Hardness     |    |                     |
| 50        | A1 LF750D  | MOCA     | 95           | 74 | 55                  |
|           |            | E300     | 95           | 74 | 42                  |
|           |            | ET5      | 95           | 73 | 37                  |
|           |            | ET10     | 96           | 74 | 41                  |
|           |            | EP10     | 97           | 73 | 42                  |
|           | B1 PHP-80D | MOCA     | 95           | 80 | 66                  |
|           |            | E300     | 99.6         | 81 | 45                  |
|           |            | ET5      | 95           | 81 | 39                  |
|           |            | ET10     | 95           | 80 | 37                  |
|           |            | EA10     | 96           | 80 | 37                  |
| 55        | C1 L325    | MOCA     | 90           | 72 | 58                  |
|           |            | E300     | 96           | 73 | 39                  |
|           |            | ET5      | 100          | 73 | 44                  |
|           |            | ET10     | 95           | 72 | 39                  |
|           |            | MOCA     |              | 75 | 43                  |
|           | D1 LFG740D | E300     | 95           | 73 | 38                  |
|           |            | ET5      | 95           | 75 | 38                  |
|           |            | EP10     | 95           | 73 | 41                  |
|           |            | MOCA     | 95           | 73 | 40                  |
|           |            | E300     | 95           | 70 | 40                  |
| 60        | E1 LW570   | MOCA     | 95           | 73 | 40                  |
|           |            | E300     | 95           | 70 | 38                  |
|           |            | ET5      | 95           | 70 | 38                  |
|           |            | EP10     | 95           | 73 | 41                  |
|           |            | MOCA     | 95           | 73 | 40                  |
|           | E2         | E300     | 95           | 70 | 40                  |
|           |            | E300     | 95           | 70 | 38                  |
|           |            | E300     | 95           | 70 | 38                  |

TABLE 1-continued

| System ID | Prepolymer | Curative | % Theory (%) | Hardness | Bashore Rebound (%) |
|-----------|------------|----------|--------------|----------|---------------------|
| E4        |            | E100     | 95           | 70       | 41                  |
| E5        |            | ET5      | 95           | 68       | 32                  |
| E6        |            | ET10     | 95           | 69       | 38                  |
| F1        | LFH120     | BDO      | 98           | 65       | 47                  |
| F2        |            | E300     | 95           | 70       | 42                  |
| F3        |            | ET5      | 99           | 67       | 34                  |
| F4        |            | ET10     | 95           | 64       | 37                  |
| G1        | 8570       | MOCA     | 95           | 73       | 30                  |
| G2        |            | E300     | 100          | 70       | 29                  |
| G3        |            | E300     | 95           | 70       | 33                  |
| G4        |            | ET5      | 95           | 72       | 31                  |
| G5        |            | EA10     | 95           | 70       | 31                  |

Samples B2, B3 and B4 were found to be brittle at 10 minutes at room temperature. Sample E2 had high viscosity and sample E3 had a longer than usual pot life. Except for sample E6, the remaining samples presented in Table 2 exhibited adequate processability.

Several samples were tested for chemical resistance or stability under CMP slurry, such as acid slurry SS12 from Cabot Microelectronics and Base Slurry Cu C2-039 from Praxair Surface Technology.

Among them, samples A2, A3, B5, C2, E5, G2 and G3 were found to be stable.

System B1 had high hardness. System E1 had high viscosity and resulted in a damping sample. High viscosity also was present in samples E5 and G4. Samples E3 and G3 were damping. Systems characterized by very low viscosity included F2 and F3.

The data indicated that aliphatic isocyanate polyether prepolymers tended to produce a solid material having a Bashore rebound lower than that of solid materials obtained using aromatic isocyanate polyether prepolymers. Adding triol, in particular at optimal levels, to the aromatic diamine tended to reduce the Bashore rebound when compared to neat aromatic diamine.

A preferred system was the very low viscosity system F3 which resulted in a material having a Bashore rebound of 34%. Also preferred were systems E5 and G2.

#### Example 2

Surfactant screening was performed using systems E5, F3 and G2. The surfactants screened were (Niax®) L-7500, L-5614, L-1580 obtained from GE Silicones; DC-193, DC-5604 and DC-5164 from Air Products and Chemicals; and DC-309, 5098EU and Q2-5211 from Dow Corning Corporation.

Results regarding foaming properties are shown in Table 2.

TABLE 2

| Surfactant | E5<br>(LW750 + ET5) | F3 (LFH120 + ET5) | G2 (8570 + E300) |
|------------|---------------------|-------------------|------------------|
| L-7500     | F                   |                   | 0                |
| L-5614     | FF                  |                   | F                |
| L-1580     | F                   |                   | FF               |
| DC-193     | FFF                 | FFF               | FFF              |
| DC-5604    | FF                  |                   | FF               |
| DC-5164    | FFF                 |                   | F                |
| DC-309     | FFF                 | FF                |                  |
| 5098EU     | FF                  |                   |                  |
| Q2-5211    | FFFF                | FFF               |                  |

where 0 indicates no foaming, F indicates some foaming and FF indicates partial foaming. FFFF and FFFFF indicate, respectively, strong foaming and very strong foaming.

As seen in Table 2, in the case of aliphatic isocyanate polyether prepolymers, DC-193 (D) and Q2-5211 (Q) produced strong or very strong foaming.

#### Example 3

10 Systems identified in Table 1 as A2, A3, B5, C2, C4, D2, D3, E5, E4, F2, F3, G2 and G4 were used for further frothing and curing testing.

First, prepolymers in each of the A2, A3, B5, C2, C4, D2, D3, E5, E4, F2, F3, G2 and G4 systems were frothed with 15 nitrogen using the surfactants, surfactant levels and conditions shown in Table 3A. Generally nitrogen flow was at 5 standard cubic feet per hour (SCFH). In Table 3A, L stands for Niax® surfactant L-1800; D for DC-193 and Q for Q2-5211 and the right hand column lists the approximate volume % 20 increase that was observed in each case.

In one illustrative example, 500 g of Adiprene® LFH120 prepolymer (melted overnight in 150° F. oven) from Chemtura was poured into a dry quart-sized tin can (de-rimmed). Then 7.5 g of DC-193 surfactant from Air Products was added 25 into the can. The can was placed onto a hot plate for heating and then equipped with a holding chain attached to a stable stand, with a copper tubing inserted into the bottom of the can for nitrogen bubbling and with a mechanical mixer with a 3" 30 propeller (see Fig. 1). The copper tubing was connected to a PE tubing from a dry nitrogen tank via a gas flow meter. The mixer was set to about 800 rpm for uniform mixing when the hot plate was on for heating the can. When the temperature in the can reached 140° F. (measured by a IR temperature gun), the mixing speed was increased to the highest setting (1500 35 rpm, measured by a tachometer) and nitrogen bubbling was turned on at 5 SCFH. The nitrogen frothing started timing and liquid level in the can was immediately measured from the top rim by a rule for frothing volume monitoring. After 45' frothing, the liquid level was measured again for the frothing 40 volume calculation (typical 30% increase). The frothed LFH120 was manually cast with different filler addition and curative within 30', kept temperature at 140° F. in an oven.

The froths were then cast and cured in the presence of the curative to produce microcellular polyurethane samples.

45 In one example, 130.8 g of the frothed LFH120 at 140° F. was poured into a dry pint tin can (de-rimmed). Started stopwatch timing and then added 35.4 g of ET5 (95% E300+5% TMP in a 500 ml brown glass bottle kept in 150° F. oven for use) into the pint can with a disposable plastic pipette in about 50 40". Immediately started to mix the mixture in the can with a 1.5" wide metal spatula for one minute, avoiding any air bubble entrapment. Poured the reaction mixture into two molds: 1" button mold and 1/16" slab mold, both pre-wiped with Stoner M800 mold release agent and pre-heated in 235° 55 F. oven before casting. Both filled molds were placed in a box oven at 235° F. The timing was closely monitored and the mixture viscosity in the can was frequently checked with the spatula until the mixture was unable to be poured for the pot life measurement (typical 6-7'). After 10', the flat portions of 60 the button samples were cut off with a utility knife to check die-cutting processability. Both button and slab samples were demolded in about 30 minutes from the mixing point. The demolded samples were placed in 235° F. oven for 16 hour postcuring. The button samples were used to measure hardness (Shore D), rebound (Bashore), density and porosity. For 65 hardness and rebound measurements, the button samples were conditioned at ambient temperature for 1+ day.

Properties of the microcellular polyurethane materials are presented in Table 3B.

As seen in the left hand column of Tables 3A and 3B, many of the combinations of prepolymer and curative identified in Table 2 are further described by surfactant type, level and/or frothing conditions. For instance the sample identified as F3-b was formed by frothing the prepolymer LFH120 with nitrogen, in the presence of DC-193 surfactant, at surfactant level of 1.5 PHR, using 1500 RPM mixing for 120 minutes; and curing the resulting froth in the presence of the curative ET5.

TABLE 3A

| Sample ID | Surfactant Type | Surfactant Level (PHR) and | Temp (° F.) | Mixing (RPM) | Frothing Time (Min) | Approximate Volume Increase (%) |
|-----------|-----------------|----------------------------|-------------|--------------|---------------------|---------------------------------|
| A2-a      |                 | 0.5 L                      | 150         | 1300         | 90-180              | 25                              |
| A2-b      |                 | 0.5 L                      | 150         | 750-1500     | 60                  | 25                              |
| A2-c      |                 | 0.5 L                      | 150         | 1500         | 90                  | 25                              |
| A2-d      |                 | 1.5 L                      | 150         | 1500         | 60                  | 30                              |
| A3-a      |                 | 0.5 L                      | 150         | 750-1500     | 60                  | 25                              |
| A3-b      |                 | 0.5 L                      | 150         | 1500         | 90                  | 25                              |
| A3-c      |                 | 1.5 L                      | 150         | 1500         | 60                  | 30                              |
| B5        |                 | 1.5 L                      | 150         | 1500         | 60                  | 30                              |
| C2        |                 | 1.5 L                      | 150         | 1500         | 60                  | 30                              |
| C4        |                 | 1.5 L                      | 150         | 1500         | 60                  | 30                              |
| D2        |                 | 1.5 L                      | 150         | 1500         | 60                  | 30                              |
| D3        |                 | 1.5 L                      | 150         | 1500         | 60                  | 30                              |
| E5        |                 | 1.5 L                      | 190-210     | 1500         | 90                  | 5                               |
| E4-a      |                 | 1.5 L                      | 190-210     | 1500         | 90                  | 5                               |
| E4-b      |                 | 1.5 Q                      | 185         | 1500         | 50                  | 35                              |
| E4-c      |                 | 1.5 D                      | 185         | 1500         | 16                  | 50                              |
| F2        |                 | 1.5 L                      | 130->100    | 1500         | 120                 | 30                              |
| F3-a      |                 | 1.5 L                      | 130->100    | 1500         | 120                 | 30                              |
| F3-b      |                 | 1.5 D                      | 140         | 1500         | 45                  | 30                              |
| G2        |                 | 1.5 D                      | 185         | 1500         | 60                  | 34                              |
| G4        |                 | 1.5 L                      | 180         | 1500         | 60                  | <5                              |

TABLE 3B

| Froth ID | Hardness Shore D | Density (g/cm <sup>3</sup> ) | Mean Pore Size (μm) | Pore Area % |
|----------|------------------|------------------------------|---------------------|-------------|
| A2-a     | 65               | 0.90                         | 30-40               | 15-20       |
| A2-b     | 67               | 0.99                         | 62                  | 15.2        |
| A2-c     | 67               | 0.98                         | 66                  | 14.2        |
| A2-d     | 66               | 0.90                         | 71                  | 20.3        |
| A3-a     | 67               | 0.99                         | 67                  | 15.5        |
| A3-b     | 67               | 0.98                         |                     |             |
| A3-c     | 65               | 0.89                         | 66                  | 20.8        |
| B5       | 65               | 0.79                         | 59                  | 27.3        |
| C2       | 57               | 0.77                         | 63                  | 27.7        |
| C4       | 56               | 0.75                         |                     |             |
| D2       | 56               | 0.80                         | 57                  | 28.8        |
| D3       | 56               | 0.80                         |                     |             |
| E4-a     | 67               | 1.01                         |                     |             |
| E4-b     | 57               | 0.74                         |                     |             |
| E4-c     | 54               | 0.66                         | 106.2               | 31.2        |
| F2       | 57               | 0.85                         | >100                |             |
| F3-a     | 56               | 0.86                         |                     |             |
| F3-b     | 61               | 0.96                         | 87.2                | 18.4        |
| G2       | 53               | 0.76                         | 74.7                | 34.6        |
| G4       | 72               | 1.21                         |                     |             |

## Example 4

Frothing conditions for preparing froth compositions based on prepolymer-curable systems A2 (LF750D+E300); A3 (LF750D+ET5); F2 (LFH120+E300); and F3 (LFH120+ET5) are shown in Table 4A below. As seen in Table 4A, Samples III, V, VI and VII were not frothed.

TABLE 4A

| 5  | Sample # | Surfactant Level (PHR) and |       | Frothing Time (Min) | Volume Increase (%) |
|----|----------|----------------------------|-------|---------------------|---------------------|
|    |          | System ID                  | Type  |                     |                     |
| 10 | I        | A2                         | 0.5 L | 150                 | 1300                |
|    | II       | A2                         | 1.5 L | 150                 | 1500                |
|    | III      | A2                         | 0     | —                   | —                   |
|    | IV       | A3                         | 1.5 L | 150                 | 1500                |
|    | V        | A3                         | 0     | —                   | —                   |
|    | VI       | F2                         | 0     | —                   | —                   |
|    | VII      | F3                         | 0     | —                   | —                   |
|    | VIII     | F3                         | 1.5 D | 140                 | 1500                |
|    |          |                            |       |                     | 45                  |
|    |          |                            |       |                     | ~30                 |

15 PVP filler was incorporated into the material as follows. 100.0 g of the frothed LFH120 at 140° F. was poured into a dry pint tin can (de-rimmed) and 15.0 g of K30 PVP powder, obtained from BASF Corp., Florham Park, N.J., was added and mixed well with a 1.5" wide metal spatula for 2 minutes until uniform.

20 Stopwatch timing was begun and 26.9 g of ET5 (95% E300+5% TMP in a 500 ml brown glass bottle kept in 150° F. oven for use) was added into the pint can with a disposable plastic pipette in about 40". Mixing the mixture in the can with the 1.5" wide metal spatula for one minute, avoiding any air bubble entrapment, was immediately started. The reaction mixture was poured into two molds: 1" button mold and 1/16" slab mold, both pre-wiped with Stoner M800 mold release agent and pre-heated in 235° F. oven before casting.

25 Both filled molds were placed in a box oven at 235° F. The timing was closely monitored and the mixture viscosity in the can was frequently checked with the spatula until the mixture could not be poured for the pot life measurement (typical 6-7 minutes). After about 10 minutes, the flat portions of the 30 button samples were cut off with a utility knife to check die-cutting processability. Both button and slab samples were de-molded in about 30 minutes from the mixing point. The de-molded samples were placed in 235° F. oven for 16 hour postcuring period.

35 In addition to PVP (abbreviated as K30), the following fillers also were evaluated: fine corn starch; methyl cellulose powder, abbreviated as A15C, obtained from Dow Chemical Company; super absorbent polymer, abbreviated as SAP and obtained under the designation of Luquasorb® from BASF 40 Chemical Company; and hollow elastic polymeric microspheres, abbreviated as d42, obtained from Akzo Nobel under the designation of Expance®.

The following procedure was employed, for instance, to obtain a microcellular material that includes Expance® particles.

50 82.0 g of the frothed LFH120 at 140 F was poured into a dry pint tin can (de-rimmed) and 1.0 g of Expance® 551DE40d42 powder, obtained from Akzo Nobel was added and mixed well with a 1.5" wide metal spatula for 3 minutes, 55 until uniform. Stopwatch timing was started right before adding 22.3 g of ET5 (95% E300+5% TMP in a 500 ml brown glass bottle kept in 150° F. oven for use) into the pint can with a disposable plastic pipette in about 40 seconds. Mixing the composition in the can was started immediately using a 1.5" wide metal spatula for one minute, avoiding any air bubble entrapment. The reaction mixture was poured into two molds: 1" button mold and 1/16" slab mold, both pre-wiped with Stoner M800 mold release agent and pre-heated in 235° F. oven before casting. Both filled molds were placed in a box oven at 235° F. The timing was closely monitored and the mixture viscosity in the can was frequently checked with the spatula until the mixture could no longer be poured for the pot

60 65

life measurement (typical 6-7 minutes). After about 10 minutes, the flat portions of the button samples were cut off with a utility knife to check die-cutting processability. Both button and slab samples were de-molded in about 30 minutes from the mixing point. The de-molded samples were placed in 235° F. oven for a 16 hour postcuring step. The button samples were used to measure hardness (Shore D), rebound (Bashore), density and porosity. For hardness and rebound measurements, the button samples were conditioned at ambient temperature for 1+ day.

The button samples were used to measure hardness (Shore D), rebound (Bashore), density and porosity. For hardness and rebound measurements, the button samples were conditioned at ambient temperature for 1+ day.

Generally, Bashore rebound was measured on the solid product formed by curing the urethane prepolymer in the presence of the curative.

In some instances, Bashore rebound also could be measured reproducibly on the microcellular materials. Repeated strokes of a microcellular material that utilized LFH120 and PVP filler, for instance, gave a Bashore rebound less than 38.

Samples were combined with various fillers and filler amounts as shown in Table 4B below. Where appropriate, froth-filler mixing conditions (RPM, time in minutes and temperature in °C.) are provided. In other cases the filler was omitted, while Samples III, V, VI and VII) were combined with filler in the absence of frothing.

TABLE 4B

| Sample ID    | Filler Type | Filler Level (wt %) | Froth-Filler Mixing (RPM; min;) | Mixing Temperature (°C.) |
|--------------|-------------|---------------------|---------------------------------|--------------------------|
| I            | —           | —                   | —                               | —                        |
| II           | —           | —                   | —                               | —                        |
| III + K30    | K30         | 4.8%                | 1100; 10                        | 90                       |
| IV           | —           | —                   | —                               | —                        |
| V + K30      | K30         | 15.6                | 1400; 15                        | 65                       |
| V + starch   | Starch      | 15.5                | 1500; 10                        | 60                       |
| V + SAP      | SAP         | 15.3                | 1500; 10                        | 85                       |
| VI           | —           | —                   | —                               | —                        |
| VII          | —           | —                   | —                               | —                        |
| VII + SAP    | SAP         | 26.6                | 800; 10                         | 60                       |
| VII + A15C   | A15C        | 19.3                | Spatula; 2                      | 70                       |
| VII + starch | Starch      | 23.8                | 800; 10                         | 75                       |
| VII + K30    | K30         | 20.8                | Spatula; 3                      | 50                       |
| VII + K30    | K30         | 14.9                | 500; 5                          | 45                       |
| VIII + K30   | K30         | 10.6                | Spatula; 2                      | 60                       |
| VIII + d42   | D42         | 0.90                | Spatula; 3                      | 50                       |
| VIII         | —           | —                   | —                               | —                        |

Samples listed in Table 4B were evaluated for hardness (Shore D) and Bashore rebound. These and other properties are shown in Table 4C:

TABLE 4C

| Sample ID  | Hardness (Shore D) | Bashore Rebound (%) | Density (g/cm <sup>3</sup> ) | Mean Pore size (μm) | Pore Area % |
|------------|--------------------|---------------------|------------------------------|---------------------|-------------|
| I          | 65                 | —                   | 0.90                         | 30-40               | 15-20       |
| II         | 66                 | —                   | 0.90                         | 71                  | 20.3        |
| III + K30  | 74                 | 40                  | 1.15                         |                     |             |
| IV         | 65                 | —                   | 0.89                         |                     |             |
| V + K30    | 67                 | 36                  | 0.93                         |                     |             |
| V + starch | 70                 | 33                  | 0.86                         |                     |             |
| V + SAP    | 64                 | 40                  | 1.05                         |                     |             |
| VI         | 70                 | 42                  |                              |                     |             |
| VII        | 67                 | 34                  |                              |                     |             |
| VII + SAP  | 70                 | 27                  | 1.17                         |                     |             |
| VII + A15C | 60                 | 44                  |                              |                     |             |

TABLE 4C-continued

| Sample ID    | Hardness (Shore D) | Bashore Rebound (%) | Density (g/cm <sup>3</sup> ) | Mean Pore size (μm) | Pore Area % |
|--------------|--------------------|---------------------|------------------------------|---------------------|-------------|
| VII + starch | 72                 | 30                  | 1.20                         | 45.6                | 30.2        |
| VII + K30    | 66                 | 43                  |                              | 48.7                | 23.3        |
| VII + K30    | 70                 | 28                  | 1.05                         | 65.2                | 39.1        |
| VIII + K30   | 61                 | 35                  | 0.89                         | 39.6                | 33.9        |
| VIII + d42   | 50                 | 30                  | 0.73                         | 87.2                | 18.4        |
| VIII         | 61                 | 37                  | 0.96                         |                     |             |

Sample III+K30 did not appear to have enough filler. Small uniform fillers but believed not to be dense enough were seen in sample V+starch, while sample V+SAP showed a broad filler distribution not dense enough. Uniform solids with not enough filler were observed in the case of samples VII+SAP and VII+starch. Both starch and SAP appeared to dissolve in the case of sample V and sample VII. Sample VII+A15C showed big cavities. As seen in the case of Sample VIII, PVP produced a microcellular material with a desired hardness and Bashore rebound.

While this invention has been particularly shown and described with references to preferred embodiments thereof, it will be understood by those skilled in the art that various changes in form and details may be made therein without departing from the scope of the invention encompassed by the appended claims.

What is claimed is:

1. A method for producing a CMP pad, the method comprising:
  - a) frothing an aliphatic isocyanate polyether prepolymer with an inert gas, in the presence of a polysiloxane-polyalkyleneoxide surfactant, to form a froth;
  - b) combining the froth with a filler soluble in a CMP slurry to form a mixture;
  - c) forming a primary pore size distributed within the pad body;
  - d) forming a secondary pore size distributed along a working surface of the pad, wherein the secondary pore size is different from the primary pore size; and
  - e) polymerizing the mixture in the presence of an aromatic diamine and, optionally, a triol, thereby producing the CMP pad.
2. The method of claim 1, wherein the filler is polyvinylpyrrolidone.
3. The method of claim 1, wherein the filler has a particle size that is different from a mean cell size produced by frothing.
4. The method of claim 1, wherein:
  - i) with respect to a theoretical amount, a curative that includes the aromatic diamine and the triol is in the range of from 90 to 105%;
  - ii) based on the total weight of a curative including the aromatic diamine and the triol, the triol is present in the curative in an amount within the range of from 0.2 to 15 weight %;
  - iii) the surfactant is present in an amount within the range of from 0.3 to 5 wt % based on the total weight of prepolymer and surfactant; or
  - iv) based on the total weight of prepolymer, surfactant, filler and curative, the filler is present in an amount within the range of from about 1 to about 20 wt %.
5. The method of claim 1, wherein the aliphatic isocyanate is selected from the group consisting of hydrogenated methylene diphenyl diisocyanate, hexamethylene diisocyanate, isophorone diisocyanate and any combination thereof.

## 21

6. The method of claim 1, wherein, a solid product formed by curing the aliphatic isocyanate polyether prepolymer in the presence of a curative that includes the aromatic diamine and the triol has a Bashore rebound that is less than 38%.

7. The method of claim 1, wherein the froth is cured at a temperature within the range of from about 50 to about 250° F.

8. A method for producing a microcellular polyurethane pad, the method comprising:

- a) frothing a urethane prepolymer to form a froth;
- b) combining the froth with a filler that is soluble in a CMP slurry to form a mixture; and
- c) forming a primary pore size distributed within the pad body;
- d) forming a secondary pore size distributed along a working surface of the pad, wherein the secondary pore size is different from the primary pore size; and
- e) curing the mixture in the presence of a curative, thereby producing the microcellular polyurethane pad, wherein, a solid product formed by polymerizing the urethane prepolymer in the presence of the curative has a Bashore rebound less than 38%.

9. The method of claim 8, wherein the curative includes an aromatic diamine and a triol.

10. The method of claim 8, wherein the urethane prepolymer is an aliphatic isocyanate polyether prepolymer or a polyester urethane prepolymer.

11. The method of claim 8, wherein the urethane prepolymer is frothed with dry air or with an inert gas selected from the group consisting of nitrogen, helium, argon, and any combination thereof in the presence of a surfactant.

12. The method of claim 8, wherein the froth is cured at a temperature within the range of from about 50 to about 250° F.

## 22

13. The method of claim 8, wherein the filler is PVP having a mean particle size that is different from a mean cell size produced by frothing.

14. The method of claim 8, wherein the microcellular polyurethane material has a Shore hardness in the range of from about 30 D to about 80 D.

15. The method of claim 8, wherein the microcellular polyurethane material has a density in the range of from about 0.5 to about 1.2 g/cm<sup>3</sup>.

16. A method for producing a CMP pad, the method comprising:

- a) frothing an aliphatic isocyanate polyether prepolymer with an inert gas, in the presence of a polysiloxane-polyalkyleneoxide surfactant, to form a froth;
- b) combining the froth with a filler soluble in a CMP slurry to form a mixture; and
- c) polymerizing the mixture in the presence of an aromatic diamine and a triol, thereby producing the CMP pad;
- d) forming a primary pore size distributed within the pad body;
- e) forming a secondary pore size distributed at a working surface of the pad, wherein the secondary pore size is different from the primary pore size;

wherein, a solid product formed by curing the aliphatic isocyanate polyether prepolymer in the presence of a curative that includes the aromatic diamine and the triol has a Bashore rebound that is less than 38%.

17. The method of claim 16, wherein the filler is polyvinylpyrrolidone.

18. The method of claim 16, wherein the filler has a particle size that is different from a mean cell size produced by frothing.

\* \* \* \* \*